

Jan. 12, 1932.

L. SILVERMAN

1,841,159

METHOD OF MAKING TEXTILE FABRICS

Filed Dec. 15, 1930



INVENTOR.

LEO SILVERMAN

BY

*Leonard L. Kalish*  
ATTORNEY.

## UNITED STATES PATENT OFFICE

LEO SILVERMAN, OF ELKINS PARK, PENNSYLVANIA, ASSIGNOR, BY MESNE ASSIGNMENTS, TO LEO SILVERMAN & CO., INC., OF PHILADELPHIA, PENNSYLVANIA, A CORPORATION OF PENNSYLVANIA

## METHOD OF MAKING TEXTILE FABRICS

Application filed December 15, 1930. Serial No. 502,448.

My invention relates to a new and useful method of making textile fabrics, whereby a certain new and highly desirable knitted millinery and trimming fabric is produced.

5 My invention relates more particularly to a novel method of forming a millinery and trimming fabric of wide sheets or webs of glycerinated regenerated cellulose, sometimes known commercially under the trade name 10 of "cellophane", whereby not only a highly desirable resultant product may be obtained, but whereby also the product may be produced with the least amount of damage or spoilage.

15 It is an object of my present invention to produce a millinery and trimming fabric having metallic lustre and pearl-like and open texture, which will be sufficiently pliant and resilient and yet permanent and durable, 20 so as to be adaptable for millinery and trimming purposes, and which will possess a thickness of body dependent upon the width of the regenerated cellulose webs, and in which the width of webs is disposed trans- 25 versely of the plane of the fabric, thereby producing at the same time, a relatively open texture.

With the above and other objects in view, which will appear more fully from the following detailed description, my invention 30 consists of a novel process or method, including a certain series and sequence of steps, whereby a relatively wide web or sheet of relatively fragile regenerated cellulose may 35 be transformed into a unique and highly useful knitted millinery and trimming fabric, without incurring damage to the regenerated cellulose or the resultant product.

40 My invention further consists of other novel features of method and product, which will appear more fully hereinafter.

45 For the purpose of illustrating my invention, I have shown in the accompanying drawings a form of apparatus which is at present preferred by me in carrying out a part of the novel method comprising my invention, since the same has been found in practice to give satisfactory and reliable results, although it is to be understood that the various instru- 50 mentalities of which my invention consists

can be variously arranged and organized, and that my invention is not limited to the precise arrangement and organization of these instrumentalities as herein shown and described.

55 Referring to the drawings in which like reference characters indicate like parts:

Figure 1 represents a diagrammatic side elevational view of the apparatus which may be used for subdividing the wide regenerated cellulose webbing into the narrower webbings for the subsequent steps of my method.

Figure 2 represents a diagrammatic plan view of the same.

Figure 3 represents a section on line 3—3 65 of Figure 1.

In carrying out my invention I utilize a web 1 of regenerated cellulose about .0007 to .003 of an inch thick and about an inch and a half to two inches wide, more or less;— 70 a suitable length of which is arranged upon a suitable roll 2. The wide regenerated cellulose web 1 is passed through opposed and operatively aligned series of circular discs 3 and 4 which are revolved in opposite directions by any suitable means (not shown). The discs 3 and 4 are arranged as indicated particularly in Figure 3, so that their contiguous edges shear or slit the web 1 along suitably spaced parallel lines, thereby dividing the web 1 into a corresponding series of narrower webs 5 of any desired width, ranging from one sixty-fourth to three sixty-fourths or a sixteenth of an inch. These narrow webs 5 are then taken up individually upon suitable take-up spools 6, driven by any suitable means.

80 The regenerated cellulose web 1 is transparent, colorless or undyed as will be brought out more in detail hereinafter.

85 The narrow, colorless regenerated cellulose webs 5 are then rewound onto suitable bobbins (not shown), and while being thus rewound, (by any suitable winding means) they are coated with a film of suitable thin oil or an oily substance, such as glycerine, for the purpose of rendering the same more susceptible to the subsequent softening operation.

90 The narrow regenerated cellulose webs thus 100

- finally wound on bobbins, are then formed into a textile fabric by knitting said webs in a moist or damp atmosphere, either singly or in multiple, over a set of knitting needles (upon any suitable machine) continuously and in the same direction, so that the tension on said regenerated cellulose web or webs is not momentarily increased at intervals, as by a change of the direction of traverse of the thread carrier with respect to the needles. Thus, the regenerated cellulose webs are knitted either singly or in multiple, over a circular knitting machine, into a tubular fabric, with the rate and direction of traverse maintained generally constant. The moisture is supplied preferably by blowing a fine spray of cold water into the atmosphere surrounding the knitting needles;—or if desired, the regenerated cellulose webs may be passed through water or vapor preliminary to the knitting. The oily film or glycerine causes a greater retention of moisture by the regenerated cellulose web, and aids in softening the same.
- 25 The tubular fabric thus produced is preferably "taken up" entirely by the weight of the fabric itself, without any additional take-up means, whereby the fabric, and hence the loops upon the needles, are not subjected to any substantial tension, so that the formation of the loops of the narrow regenerated cellulose webs is maintained free of all strain or tendency to crush or distort the loops, or to sharply bend said webs beyond the curvatures 30 which the regenerated cellulose webs tend normally to assume by reason of the inherent resiliency of said webbing.
- 35 The raw tubular knitted fabric, thus produced, is then washed while in the tubular formation or condition, to remove the oily film on the regenerated cellulose web, and while still in the tubular formation or condition, the fabric is dyed to the desired color.
- 40 While still in the tubular formation or condition the dyed fabric is then dehydrated centrifugally or by other suitable means, to a point where it still contains a substantial percentage of moisture;—about 5%, more or less, and is then drawn onto a suitable form, upon 45 which the fabric is stretched out. The fabric is allowed to dry in the air by normal evaporation. Lastly the tubular formation is cut open longitudinally, so that a flat, single-ply 50 finished web of fabric is produced.
- 55 The fabric thus produced possesses a pearl-like and open texture and a metallic lustre, and is capable of withstanding sufficient wear to make it highly useful for millinery and trimming purposes.
- 60 I am aware that the invention may be embodied in other specific forms without departing from the spirit or essential attributes thereof, and I therefore desire the present embodiments to be considered in all respects as 65 illustrative and not restrictive, reference

being had to the appended claims rather than to the foregoing description to indicate the scope of the invention.

Having thus described my invention, what I hereby claim as new and desire to secure by Letters Patent, is:

1. The method of making a millinery and trimming fabric which consists in slitting a long and relatively wide web of regenerated cellulose into long and relatively narrow webs of a width ranging from approximately one sixty-fourth of an inch to approximately one-sixteenth of an inch, depending upon the thickness desired in the resultant fabric; softening said relatively narrow webs, forming the same into a tubular textile fabric, by knitting said relatively narrow webs over a set of knitting needles continuously and in the same direction, thereafter dyeing said tubular knitted fabric and dehydrating the same, and cutting open said tubular formation longitudinally to form a finished, flat web of knitted fabric.

2. The method of making a millinery and trimming fabric which consists in cutting a long and relatively wide web of regenerated cellulose into correspondingly long, but relatively narrow webs of a width ranging from approximately one sixty-fourth of an inch to approximately one-sixteenth of an inch, depending upon the thickness desired in the resultant fabric, softening said relatively narrow webs, forming the same into a tubular textile fabric, by knitting said relatively narrow webs over a set of knitting needles continuously and in the same direction, and lastly cutting open said tubular formation longitudinally to form a finished, flat web of knitted fabric.

3. The method of making a millinery and trimming fabric which consists in cutting a long and relatively wide web of regenerated cellulose into correspondingly long but relatively narrow webs of suitable width, depending upon the thickness desired in the resultant fabric; softening said relatively narrow webs, forming the same into a tubular textile fabric, by knitting said relatively narrow webs over a set of knitting needles continuously and in the same direction with the width of said narrow webs disposed generally transversely of the plane of the resultant fabric, thereafter dyeing said tubular knitted fabric and dehydrating the same, and cutting open said tubular formation longitudinally to form a finished, flat web of knitted fabric of open texture.

4. The method of making a millinery and trimming fabric which consists in cutting a long and relatively wide web of regenerated cellulose into correspondingly long, but relatively narrow webs of suitable width, depending upon the thickness desired in the resultant fabric, softening said relatively narrow

webs, forming the same into a tubular textile fabric, by knitting said relatively narrow webs over a set of knitting needles continuously and in the same direction, with the 5 width of said relatively narrow webs disposed generally transversely of the plane of the resultant fabric, and lastly cutting open said tubular formation longitudinally to form a finished, flat web of knitted fabric.

10 5. The method of making a millinery and trimming fabric which consists in cutting a long and relatively wide web of regenerated cellulose into correspondingly long, but relatively narrow webs of suitable width, depending 15 upon the thickness desired in the resultant fabric, treating said relatively narrow webs with a softening reagent, forming said cut webs into a tubular fabric, by knitting the same over a set of knitting needles generally continuously and in the same direction with the width of said relatively narrow webs disposed generally transversely of the plane of the resultant fabric, and without any substantial tension on the resultant fabric issuing from said needles, thereafter dyeing 20 said tubular knitted fabric and dehydrating the same, and lastly cutting open said tubular formation longitudinally to form a finished single web of the knitted fabric.

25 6. The method of making a millinery and trimming fabric which consists in cutting a long and relatively wide web of regenerated cellulose into correspondingly long, but relatively narrow webs of suitable width, depending 30 upon the thickness desired in the resultant fabric, treating said relatively narrow webs with a softening reagent, including an oily liquid and moisture, forming said cut and softened webs into a tubular fabric, by 35 knitting the same over a set of knitting needles generally continuously and in the same direction with the width of said relatively narrow webs disposed generally transversely of the plane of the resultant fabric, 40 and without any substantial tension on the resultant fabric issuing from said needles, thereafter dyeing said tubular knitted fabric and dehydrating the same, and lastly cutting open said tubular formation longitudinally 45 to form a finished single web of the knitted fabric.

50 In testimony whereof I have hereunto set my hand and seal this 12th day of December, 1930.

55 LEO SILVERMAN.